

June 15, 1954

S. S. KISTLER  
CYLINDER AND LINER

2,681,260

Filed July 27, 1951

FIG. 1



# UNITED STATES PATENT OFFICE

2,681,260

## CYLINDER AND LINER

Samuel S. Kistler, West Boylston, Mass., assignor to Norton Company, Worcester, Mass., a corporation of Massachusetts

Application July 27, 1951, Serial No. 238,862

4 Claims. (Cl. 309—3)

1

The invention relates to cylinders and liners, especially cylinders and liners for internal combustion engines, steam engines, reciprocating pumps and sleeve bearings, and a process for making them.

Another object of the invention is to provide cylinders and cylindrical liners made out of ferrous metal, either iron or steel, having an interior "case" of metal containing a hard carbide. Another object of the invention is to provide cylinders and cylindrical liners having interior surfaces of great hardness. Another object of the invention is to provide strong cylinders and liners having hard interior surfaces. Another object of the invention is to provide cylinders and cylindrical liners having interior surfaces of great hardness due to the presence of hard carbide therein without the necessity of going to the expense of providing enough of the hard carbide to permeate all of such cylinders or liners.

Another object of the invention is to provide cylinders and cylindrical liners the bodies of which are tough and strong and the inner surfaces of which are very hard and wear resistant. Another object is to make a cylinder or cylindrical liner which is very hard on the inside but (relatively) soft on the outside so that it can be readily machined on the outside.

Other objects will be in part obvious or in part pointed out hereinafter.

The accompanying drawings are illustrative of apparatus which can be used to carry out the invention but it must be understood that other apparatus can be used, that shown being merely illustrative. In these drawings

Figure 1 is a view partly in side elevation and partly in axial section of such apparatus.

Figures 2 and 3 are sectional views taken along the lines 2—2 and 3—3 respectively of Figure 1.

Referring to Figure 1, a supporting bracket 10 is bolted to the floor by means of bolts 11. The upper end of the bracket 10 has a forked portion 12 through which extends a pin 13 which passes through a bracket 14 suitably secured to a frame 15, whereby the frame 15 is articulated to the bracket 10.

Secured to the frame 15 is an electric motor 20 having a motor shaft 21 coupled by means of a coupling 22 and keys 23 to a shaft 24 having a head 25. The head 25 is secured by bolts 26 to a circular plate 27 constituting an end plate of a cylindrical mold. Another circular plate 28 is connected to the plate 27 by means of bolts 29 having nuts 30 thereon at one end; the bolts 29 pass through the plates 27 and 28 as shown. Be-

2

tween the plates 27 and 28 and held in position by the pressure exerted on the plates by the bolts 29 is a hollow cylinder 31. Thus is formed a hollow cylindrical mold body rotatable on the axis of the cylindrical inside surface of the body. The plates 27 and 28 and the hollow cylinder 31 can be made of iron or steel.

Secured to the end of the plate 28 by means of bolts 35 is a head 36 on the end of a hollow shaft 37 which extends through a bearing 38 supported by a post 39 connected to the frame 15. I shall not describe the various parts of the bearing 38 as the drawing is clear and such details can be widely varied.

The frame 15 which as shown may have the shape of a table top can be placed in a vertical position as well as in the horizontal position in which it is shown in Figure 1. To that end a latch 40 slideable in a holder 41 which is secured to the underside of the frame 15 is engageable with a plate 42 on the top of a post 43 secured to the floor by means of bolts 44. When the frame 15 is swung into the horizontal position the latch 40 automatically operates to lock it in that position while the post 43 restrains the frame 15 from further clockwise movement.

When it is desired to place the frame 15 in a vertical position, the latch 40 is withdrawn by means of its handle 45, the frame is swung counter-clockwise and the operator steps on a plate 46 through which extends a bolt 47 having nuts 48 under the plate 46, the bolt 47 extending also through a block 49 secured to the bracket 10 and being surrounded by a spring 50 under the bolt head 51, the spring 50 acting to urge the parts into the position shown in Figure 1 but when the operator steps on the plate 46 the bolt head 51 is lowered and can enter a recess 52 at the end of the frame 15 whereby releasably to lock the frame 15 in the vertical position.

The hollow mold cylinder 31 may have any suitable liner embodied in a hollow cylindrical member 55, a solid end plate 56 and an end plate 57 having a hole therein concentric with a hole through the circular plate 28. These liner parts 55, 56 and 57 can be made out of any suitable material which is sufficiently refractory and non-reactive for the purpose intended. Sintered alumina is satisfactory and hollow tubular shapes such as the part 55 as well as disc shapes such as the parts 56 and 57 can be readily made out of sintered alumina. Liner parts made in this manner can be ground with diamond grinding wheels to produce true surfaces and then the liner parts can be used over and over again as the cast-

ing shrinks away from the part 55 in cooling and hence readily comes out. I have however successfully used a paste of 80 parts of fine alumina and 20 parts of ball clay with enough water to make it workable, the alumina being one half 600 mesh size and one half 150 mesh size. This can be hand molded in position with a spatula while turning the mold 31 and after drying makes a good mold lining which is destroyed after casting. But when casting cast iron cylinders I can use steel mold liner parts 55, 56 and 57 because the melting point of steel is considerably higher than that of cast iron.

The procedure for making the cylinders and liners may start with placing the frame 15 in the vertical position, wherefor as will readily be seen the axis of the mold body 31 will be vertical, whereupon the motor 20 is started and liquid ferrous metal 60 is poured into the hollow shaft 37 whereupon it promptly flows into the cylindrical space bounded by the liners 55, 56 and 57 and the centrifugal force spreads it out in the form of a hollow cylinder of liquid. The carbide material may be introduced into the mold with, before or after the liquid ferrous metal. The carbide material is in the form of particles (not liquid) and can be of particle size as large as 8 mesh but may also be smaller. I prefer sizes between 100-300 mesh, but I have found that precipitated carbide particles as fine as 2 microns diameter are very effective. As it is better to form the cylinder or liner in a horizontal position because thereby the component of gravity does not affect the shape, right after pouring the ferrous metal and introducing the carbide material the operator should step on the plate 48, thus withdrawing the head 51 from the recess 52, and should then swing the frame 15 rapidly to the horizontal position, whereupon the latch 49 will automatically lock it in that position which is shown in Figure 1. Rotation of the mold is continued and eventually the metal freezes usually starting at the outside and when the metal 60 has become a solid piece the motor 20 is stopped and both mold and piece are allowed to cool whereupon eventually the mold parts can be disassembled.

Optionally I may use further equipment in the process. Referring again to Figure 1, a pneumatic vibrator 70 is secured by means of flexible brackets 11 to the frame 15 and this is energized by compressed air introduced by a flexible rubber hose 72. To one end of the vibrator 70 is secured a slideway block 73 by means of bolts 74. A removable slide 75, illustrated also in Figure 2, and having a handle 76 can be inserted in the slideway block 73 from the right toward the left and when pushed to the extreme position as shown in Figure 1 a spring-pressed ball 80 releasably locks the parts together, an abutment 81 preventing further movement toward the left.

This slide 75 upholds a long T-shaped iron 85 illustrated in cross section in Figure 3 and in side elevation in Figure 1. This T-shaped iron 85 can be welded to the end of the slide 75 both parts being conveniently made of steel. At the left hand or front end of the T iron 85 is a tray 87 which can also be made of steel and welded to the T iron. This tray 87 has holes, not shown, in the bottom thereof, so it constitutes in effect a sieve, the holes being of a size just large enough to pass the particles of carbide. This tray 87 is, when using the apparatus just described, filled with carbide material and, when the frame 15 has been swung to the horizontal position, the tray 87

87 is inserted in the mold as shown, the slide 75 being inserted in the slideway block 73 as shown, whereupon the vibrator 70 is energized and thus the carbide material is slowly sifted onto the interior surface of the melt 60 which concentrates it at said interior surface whereas the difference in specific gravity of the carbide material and the iron respectively prevent the carbide material from migrating into the interior of the melt 60.

It may also introduce a special atmosphere into the rotating mold, for example an atmosphere of hydrogen, and to that end, as shown in Figures 1 and 3, I secure an iron pipe 90 to the T iron 85, this iron pipe 90 having a bend 91 with a nipple thereon at the right hand end to which a rubber hose 92 can be quickly connected to introduce the desired gas into the rotating mold.

I have found that I can make cylinders and liners of ferrous metal having at the inside surface a layer of hard carbide bonded together by the ferrous metal using carbide selected from the group consisting of vanadium carbide, titanium carbide, zirconium carbide and mixtures thereof. I can do this without dispersing the carbide throughout the metal of the cylinder or the liner. For practical purposes it is sufficient if the inside of the cylinder or liner is hard for a depth of from 2 to 40 thousandths of an inch. The amount of carbide in the interior portion containing the carbide should be between 20% and 75% by volume. It is difficult to pack the carbide particles closer than 75% in the centrifugal field, while 20% by volume appears to be a practical lower limit of concentration for effective resistance to wear.

Vanadium carbide is a compound generally assumed to be VC. However I am not to be held to the correctness of this formula and any true compound of vanadium and carbon without other elements in the compound is usable. Similarly titanium carbide is assumed to be TiC and zirconium carbide ZrC and the same provisos apply, namely that I am not to be held to the correctness of these formulae and any true compound of titanium or zirconium and carbon not containing other elements in the compound can be used.

The following table gives the hardness, melting point and specific gravity of the carbides mentioned and also of pure iron known as ferrite.

Table I

| Material                     | Hardness on the Knoop Scale of the Gram Load Indicated after the slant line | Melting Point, Degrees Centigrade | Specific Gravity at Room Temp., Water = 1 |
|------------------------------|-----------------------------------------------------------------------------|-----------------------------------|-------------------------------------------|
| Iron, ferrite.....           | 400/25                                                                      | 1,535                             | 7.85                                      |
| Iron carbide, cementite..... | 1,150/25                                                                    | 1,837                             | 7.4                                       |
| Vanadium carbide.....        | { 2,520/25<br>2,080/100 }                                                   | 2,830                             | 5.4                                       |
| Titanium carbide.....        | 2,470/100                                                                   | 3,140                             | 4.9                                       |
| Zirconium carbide.....       | 1,800/100                                                                   | 3,530                             | 6.4                                       |

The above table shows the great advantage of vanadium, titanium and zirconium carbides over iron carbide for wear resistance. It should be noted that the hardness of sapphire, which is 9 on Moh's scale, is approximately that of vanadium carbide.

All of the carbides with which I am familiar are soluble in molten iron. The degree of solubility varies greatly from one carbide to the other, however, and I find that vanadium carbide is the least soluble. I can disperse vanadium

carbide in molten cast iron or steel and centrifuge the particles to the inner surface without great loss through solution. The grains, when examined microscopically after solidification, show rounded corners and edges and there is some evidence of precipitation of vanadium carbide from the melt on solidification. To avoid dissolving the added carbide, I find it convenient, though somewhat expensive, to add approximately 2% of vanadium as ferrovanadium to the melt. This saturates the melt sufficiently with vanadium carbide, formed by reaction with the carbon of cast iron and steel, so that added carbide does not appear to dissolve. The question whether or not to add the vanadium is an economic one to be determined by circumstances.

Among the very hard carbides with specific gravity sufficiently low to concentrate in the inner surface on centrifuging, the other two that I have found useful are titanium and zirconium carbides. They are both of limited solubilities in molten cast iron or steel. The solubility depends greatly upon the temperature and therefore there is an advantage to working with the lowest temperature at which the metal is fluid. Titanium and zirconium carbides mixed into a melt have the property of increasing its viscosity very greatly and therefore decreasing the ease of centrifuging to the inner surface. If a large excess of melt is used, the viscous effect of these carbides can be overcome but loss of carbide through solution then becomes excessive. I have therefore found that it is most convenient to sprinkle these carbides onto the surface of the molten iron or steel after it has started to spin in the mold and thus there is no tendency for them to mix throughout the melt and the viscous effect gives no trouble.

The character of the atmosphere is particularly important when titanium and zirconium carbides are used and I have found that it is desirable to use either high vacuum or pure, dry hydrogen. The latter is more convenient and has proved adequate.

Apparently when the atmosphere is not thoroughly purified, the titanium or zirconium carbide develops a thin oxide film on its surface that interferes with wetting by the metal. I have overcome this difficulty when using tank hydrogen, which contains some moisture, by first compressing the titanium or zirconium carbide with more than an equal volume of iron powder into pellets and sintering these in pure hydrogen. I have customarily used about 25 tons per square inch for pressing the pellets. By this means the surfaces of the carbide particles are made to adhere to the iron and when these particles are floated on the surface of a melt, the iron goes into solution, or melts, and the carbide grains are freely wetted and spread over the molten surface by centrifugal force.

The carbides do not need to be added as such to steel or cast iron but can be generated in situ and concentrated in the inner surface by centrifuging. In order to generate the carbides in the melt, enough ferrovanadium, ferrotitanium or ferrozirconium may be added more than to saturate the melt so that carbide particles will precipitate before solidification occurs. In this case the carbide particles are usually quite small and migrate slowly toward the inner surface so that it is desirable to use a relatively high centrifugal force, e. g., 100×gravity.

A precaution has to be observed in generating the carbide in situ to see that there is enough

carbon in the melt to produce the carbide plus providing the properties of the melt desired.

Instead of mixing the ferro alloys with the melt, it is convenient to spread them on the inner surface during centrifuging and thus concentrate them where they are desired and therefore not waste alloy by distributing it throughout the whole melt. I have found it desirable in some cases to mix some carbon with the ferro alloy to help in converting it to carbide on the inner surface during casting. Instead of adding vanadium, titanium or zirconium or mixtures thereof as ferro alloys, I may add any of them or a mixture of two or all three in the form of metal powder, relatively pure. Such metal powder may be mixed with carbon powder or not, depending on the amount of carbon otherwise available.

#### Example 1

20 I mixed 4 grams of 200 mesh vanadium carbide with 40 grams of cast iron chips, melted these together at a temperature of about 1250° C. and cast the melt into a spinning mold at the same temperature using an atmosphere of hydrogen. 25 The mold liner 55 was one and five-eighths inches inside diameter by one inch long and was spun at 1200 R. P. M. On cooling and sectioning the cylinder thus cast, the vanadium carbide was found to have concentrated in the inner surface 30 of the cylinder. The grains showed some evidence of solution in the cast iron and there were granules of vanadium carbide in the cast iron produced by precipitation on cooling, showing that some of the vanadium carbide dissolved but not 35 enough to prevent a satisfactory armoring of the inner surface.

#### Example 2

Pellets were molded from a mixture of 4 grams vanadium carbide, 40 grams of a granular cast iron alloy, known to the trade as NiHard, and 1.6 grams of a 50% ferrovanadium using a pressure of 25 tons per square inch. These were placed in a mold of the same size as Example 1 and melted by inductively heating the mold to a temperature of 1300° C. while it was spinning at 1200 R. P. M. It was allowed to cool to 1000° before spinning stopped. In this case the vanadium carbide particles were found concentrated at the inner surface and there was no evidence of solution. The entire mass of cast iron outside of the vanadium carbide layer contained numerous very fine particles of vanadium carbide too small to migrate rapidly in the centrifugal field and therefore only a fraction of them had reached the inner surface before solidification. These were produced by precipitation of VC from solution due to the reaction between the added vanadium and carbon in the cast iron.

#### Example 3

Pellets similar to those in Example 2 were molded but without the vanadium carbide. These were placed in a mild steel mold of the dimensions given in Example 1 and melted at 1300° C. while rotating at 1200 R. P. M. The temperature was lowered slowly at the rate of about 10° per minute to 1150° after which the heat was turned off and the motor stopped when the temperature reached 1000°. The cross section of the cylinder formed showed great numbers of very fine vanadium carbide particles concentrated in the inner surface of the cylinder. Many vanadium carbide particles were also to be found throughout the mass showing that they are so small as to sediment only slowly in the melt.

## Example 4

A mold of the same dimensions as in Example 1 was heated by induction to 1250° C. and 50 grams of melted gray cast iron poured in. Onto the surface of this rotating molten cast iron was sprinkled 3 grams of 200 mesh vanadium carbide. The atmosphere used was tank hydrogen. On cooling, the vanadium carbide was found to have been thoroughly wetted by the cast iron and to have concentrated in the inner surface of the cylinder. This mold was also rotated at 1200 R. P. M.

## Example 5

Molten cast iron was spun in a mold as in Example 4 but 4 grams of 50% ferrovanadium was spread on the surface instead of vanadium carbide. On cooling, the inner surface was found to be heavily loaded with fine vanadium carbide particles produced by reaction of ferrovanadium with the carbon in the cast iron.

## Example 6

The same procedure was used as in Example 4 only 6 grams of titanium carbide were used. After heating to 1300° C. and cooling, titanium carbide was found imbedded in the inner surface in sufficient quantity to give it great hardness and wear resistance.

## Example 7

The procedure followed in Example 4 was used except zirconium carbide was substituted for the vanadium carbide, using a well purified hydrogen atmosphere. On sectioning the cylinder, the zirconium carbide was found well imbedded in the inner surface.

## Example 8

A cylinder of mild steel was made with inside dimensions 1 1/8" diameter by 1" long. On the inner surface was spread a paste of 4 grams of 200 mesh vanadium carbide and 1 gram of fine graphite mixed with glycerin. This was rotated at 1200 R. P. M. in an atmosphere of hydrogen and heated by induction to 1250° C. On cooling, it was found that the carbon had fused the inner surface of the cylinder to a depth of 1 to 2 mm. and the vanadium carbide had been imbedded in this layer. The alloy on the inner surface consisted mainly of cementite and ferrite.

## Example 9

The procedure was followed as in Example 8 only 10.2 grams of 50% ferrovanadium and 1.7 grams of fine graphite were spread on the inner surface, using glycerin as a vehicle. When heated to 1260° C. and cooled, the inner surface was found to be armor plated to a depth of 1 mm. with vanadium carbide dispersed in iron.

## Example 10

Pellets were made by mixing 60 parts by weight of powdered iron with 40 parts of 200 mesh titanium carbide and pressing in a mold at 25 tons per square inch. Ten grams of these pellets were broken up to about 8 mesh size and distributed over the inner surface of a cold cast iron cylinder in a mold rotating at 1200 R. P. M. Using an atmosphere of purified and dried hydrogen, the mold was heated inductively to a temperature of 1300° C. and allowed to cool. The iron-titanium carbide pellets were found to have completely disintegrated and the titanium carbide grains to be well distributed and thoroughly imbedded throughout the inner surface of the cylinder.

## Example 11

The procedure was followed as in Example 8 only titanium carbide was substituted for vanadium carbide. With a good hydrogen atmosphere the titanium carbide imbedded satisfactorily in the inner surface of the iron cylinder.

## Example 12

A cylinder was cast of "NiHard" cast iron. While still at a temperature of approximately 1300° C. a mixture of 3 grams of metallic titanium in granular form and .8 gram of fine graphite were sprinkled onto the molten surface. On cooling, it was found that the inner surface of the cast iron was filled with fine titanium carbide particles.

## Example 13

I mixed 30 grams of cast iron chips, 2 grams of titanium shavings and 0.6 gram of fine graphite and spread in a cold rotating mold of mild steel like described in Example 1. The speed was 1200 R. P. M. I then inductively heated the mold rapidly to 1300° C. and held between 1300° C. and 1310° C. for six minutes whereupon I turned off the current. The atmosphere was tank hydrogen. On sectioning, polishing and examining under the microscope, the inner surface was found to contain great numbers of TiC particles, ranging from 2 to 6 microns in diameter, to a depth of about a millimeter.

The atmosphere in which the centrifugal forming of a hard inner surface on a metal cylinder is carried out may vary considerably depending on the carbide to be used. For example, burnt gas such as exhaust from a gasoline engine when the carburetor is set for excessive gasoline, or that known to the trade as "Endogas" is perfectly satisfactory for the introduction of vanadium carbide into the surface. Pure nitrogen, carbon monoxide or mixtures of these gases may also be used, as well as mixtures containing hydrogen, which is an important constituent of the "Endogas." When it is desired to use zirconium or titanium carbide, I have found it preferable to use a very carefully dried gas free from any oxygen and I prefer pure hydrogen. The inert gases, such as helium and argon, may be used but precautions necessary to eliminate all oxygen or water vapor are troublesome.

A high vacuum is, under some circumstances, the best "atmosphere" but its inconvenience dictates that for practical purposes one of the above-named gases should be used. The gases may be introduced through the rubber hose 92 and pipe 90. The various gases mentioned are non-oxidizing.

The advantages of the invention lie in the fact that the manufacturing process is relatively simple and only a small amount of the expensive carbide material need be used. All three of these carbides usable in the invention are expensive. Furthermore the major portion of the cylinder or liner made according to my invention has little or none of the carbide or carbides of vanadium, titanium or zirconium and hence is readily machinable and also stronger and tougher than it would be if it contained a large percentage of such carbide or carbides.

I use the terms ferrous metal and ferrous melt with the same meanings in which they are now generally used in industry that is to say to apply to materials selected from the group consisting of iron and steel. By iron of course is included

so-called cast iron whether gray iron or white iron, also malleable iron. By steel I mean to include everything which is commonly called steel and the art gives the term a rather definite meaning although to define it may take many words. The steels of course include electric furnace steels, open hearth steels, bessemer steels and stainless steel. Steels generally contain some iron carbide as cementite and little if any free carbon as graphite whereas the cast irons may contain such free carbon as graphite. Many elements have been added to iron to make the various steel alloys and it is impossible for me even to give a list of all the known steel alloys. Metals usually added to iron to make steel alloys include chromium, cobalt, manganese, molybdenum, nickel, silicon, tungsten and vanadium.

While in many cases especially when the carbide particles are added by means of the tray 87 it is sufficient to rotate the mold at an angular velocity sufficient to form a cylindrical inner surface on the melt, in some cases forces up to or above 100g (where g is the force of gravity and equivalent to 32 feet per second per second acceleration) are preferably used. These are easy to attain as can be readily calculated from the equation  $v^2 = Gr$ , where  $v$  is peripheral velocity in feet per second, G is centrifugal force in terms of feet per second per second and  $r$  is the radius of the periphery or point involved in feet. For example with a motor speed of 1200 R. P. M.  $G = 41g$  at a radius of one inch,  $G = 82g$  at a radius of two inches and  $G = 123g$  at a radius of three inches. With a motor speed of 3000 R. P. M.  $G = 256g$  at a radius of one inch and  $G = 512g$  at a radius of two inches etc. The only limiting factor, therefore, is the strength of the mold and steel mold cylinders 31 of inside diameters up to six inches and more can readily be made which will stand centrifugal force up to and beyond 1000g. Especially when mixing the carbide with the ferrous melt or forming the carbide in situ but even also in those cases where I add the carbide to the rotating mold and deposit it on the inner surface of a ferrous melt I prefer to keep the ferrous metal molten and to maintain the mold rotating at an angular velocity equivalent to at least 10g for at least twenty seconds with the carbide or elements thereof present.

With a force many times that of gravity a slight difference in specific gravity will be sufficient to cause the lighter carbide particles to move quickly to the interior of the rotating melt. Indeed angular velocities much lower than 1200 R. P. M. can be used. Most of the elements for making alloy steels above listed have specific gravities greater than those of the three carbides selected as shown in the following table.

Table II

| Elements for Making Alloy Steels | Specific Gravity at Room Temp., Water = 1 | 70 |
|----------------------------------|-------------------------------------------|----|
| Chromium                         | 7.1                                       |    |
| Cobalt                           | 8.9                                       |    |
| Manganese                        | 7.2                                       |    |
| Molybdenum                       | 10.2                                      |    |
| Nickel                           | 8.9                                       |    |
| Silicon                          | 2.42                                      |    |
| Tungsten                         | 19.3                                      |    |
| Vanadium                         | 5.87                                      |    |

It will be seen from the above table that any of these elements for making alloy steels can be used in considerable quantity while still main-

taining the specific gravity of the melt 60 above the specific gravity of the carbide particles. Even with silicon, the lightest element in the table, the largest quantity used commercially in a structural alloy is 14.5% in "Duriron" and this has a specific gravity of 7.0, substantially above that of the carbides used. Usually silicon is used in very much smaller quantities in alloys of still higher specific gravities.

Articles made in accordance with the invention may be hollow cylinders and at least the interior surface will be cylindrical, but the exterior surface can be conical or stepped or otherwise depart from a true cylindrical surface. At the 15 inner surface of such articles there is a layer at least .002 inch thick consisting of carbide and ferrous metal, the carbide being selected from the group consisting of vanadium carbide, titanium carbide and zirconium carbide and mixtures thereof, the carbide being present in the interior layer to the extent of from 20% to 75% by volume. For reasons heretofore explained, the major portion of the articles will be ferrous metal containing not over 5% by volume of the aforesaid carbide.

After the hollow article is made as above indicated the interior thereof is ground preferably with a diamond grinding wheel or it is honed with a honing tool having diamond abrasive sticks. In this manner a smooth surface is provided on the inside of the article so that it can be used as a cylinder or a liner for an internal combustion engine, a bearing, a pump cylinder, etc.

Accordingly the process involves providing a rotatable mold, mounting the mold for rotation on an axis, providing in the mold a melt of ferrous metal and material including matter selected from the group consisting of vanadium, titanium, zirconium and complexes thereof, rotating the mold to form an interior cylindrical surface on the melt and at an angular velocity to maintain at the inner surface centrifugal force equivalent to at least 10g for at least twenty 35 seconds and maintaining the rotation of the mold at an angular velocity and for a length of time sufficient to insure the presence of enough of such material to provide, after solidification, carbide selected from the group consisting of vanadium carbide, titanium carbide, zirconium carbide and mixtures thereof to an extent of at least 20% by volume for a depth of at least .002 inch at the inner surface. Vanadium matter includes vanadium metal, ferrovanadium and vanadium carbide, titanium matter includes titanium metal, ferrotitanium and titanium carbide and zirconium matter includes zirconium metal, ferrozirconium and zirconium carbide. I use the word "complexes" instead of "mixtures" because I want to include compounds as well as mixtures.

In Examples 8, 9, 10, 11, 12 and 13, the iron or steel of the cylinder or of the added ferrous metal or both was melted so that in all of the examples there was ferrous melt in the mold while it was rotating. In all of the examples I actually kept the mold rotating at the specified angular velocity and at the specified temperature for minimum of half a minute, but a lesser period will be satisfactory as indicated.

The apparatus is illustrative and the mold might be maintained horizontal at all times using a short hollow shaft 37 and introducing the melt in the form of a stream through the shaft or otherwise proceeding according to any of the examples or according to any part of the descrip-

tion. In many cases an inductively heated mold may be used.

It will thus be seen that there has been provided by this invention cylinders and liners and a process for producing the same in which the various objects hereinbefore set forth together with many thoroughly practical advantages are successfully achieved. As many possible embodiments may be made of the mechanical features of the above invention and as the art herein described might be varied in various parts, all without departing from the scope of the invention, it is to be understood that all matter hereinabove set forth, or shown in the accompanying drawings, is to be interpreted as illustrative and not in a limiting sense.

I claim:

1. A hollow article having an interior cylindrical surface, said hollow article being made of ferrous metal selected from the group consisting of iron and steel and having at the interior surface thereof a layer at least .002 inch thick consisting of carbide and said ferrous metal, said carbide being selected from the group consisting of vanadium carbide, titanium carbide and zirconium carbide and mixtures thereof, said car-

bide being present in said interior layer to the extent of from 20% to 75% by volume, the major portion of said hollow article containing not more than 5% by volume of said carbide.

2. A hollow cylinder according to claim 1, in which the carbide is vanadium carbide.

3. A hollow cylinder according to claim 1, in which the carbide is titanium carbide.

4. A hollow cylinder according to claim 1, in which the carbide is zirconium carbide.

References Cited in the file of this patent

UNITED STATES PATENTS

| Number    | Name        | Date          |
|-----------|-------------|---------------|
| 1,346,188 | Fahrenwald  | July 13, 1920 |
| 2,166,634 | Lessage     | July 18, 1939 |
| 2,222,525 | Zink        | Nov. 19, 1940 |
| 2,273,614 | Batie       | Feb. 17, 1942 |
| 2,292,662 | Sanders     | Aug. 11, 1942 |
| 2,400,495 | Ford et al. | May 21, 1946  |
| 2,461,765 | Olt         | Feb. 15, 1949 |

FOREIGN PATENTS

| Number  | Country       | Date           |
|---------|---------------|----------------|
| 643,435 | Great Britain | Sept. 20, 1950 |